

Patented July 15, 1941

2,249,175

# UNITED STATES PATENT OFFICE

2,249,175

## PREPARATION OF SOLUTIONS OF HEAT- RIPENED CELLULOSE XANTHATE

George A. Richter and Harold P. Vannah, Berlin,  
N. H., assignors to Brown Company, Berlin,  
N. H., a corporation of Maine

No Drawing. Application October 17, 1938,  
Serial No. 235,458

3 Claims. (CL 260—217)

This invention relates to the preparation of solutions of heat-ripened cellulose xanthate. It deals with a process by which cellulose xanthate is ripened quickly under heat and is then put into the form of a finished cellulose xanthate or viscose solution of the desired characteristics, including cellulose content, causticity, degree of ripeness, ripeness-stability, etc., for the particular purpose in view, for instance, for spinning into rayon filaments or casting into films.

In accordance with the present invention, cellulose xanthate of a cellulose content or concentration greater than that of the finished cellulose xanthate or viscose solution to be produced is heated to much higher than room temperature until the xanthate has acquired substantially the degree of ripeness desired, whereupon the heated xanthate is admixed with relatively cold or refrigerated aqueous medium in amount sufficient to dilute the cellulose content of the xanthate to that of the final solution to be produced. The aqueous medium thus admixed with the heated xanthate is sufficiently cold or refrigerated to arrest rapidly further substantial ripening reaction in the xanthate. Its admixture with the xanthate is effected in the presence of alkali in amount to promote substantially complete dissolution of the xanthate in the aqueous medium, thereby conducting to the desired finished cellulose xanthate or viscose solution.

The cellulose xanthate to be heat-ripened pursuant to the present invention may be a cellulose xanthate solution of distinctly higher cellulose content than that of the final solution desired, for instance, a finished solution such as is to be spun into rayon filaments. Thus, when the finished solution is to have a cellulose content of about 7%, the solution to be heat-ripened by the process hereof may have a cellulose content upwards of, say, 8% as a minimum. Immediately after the heat-ripening treatment, the solution may be diluted to the desired final cellulose content with an appropriate amount of water sufficiently cold or refrigerated to arrest at once any further substantial ripening reaction and to yield a finished solution at a temperature sufficiently low to permit keeping of the solution for a substantial period of time without material change in ripeness. Again, the cellulose xanthate subjected to the heat-ripening treatment hereof may be in the form of the usual xanthated crumbs such as undergoes dissolution in weak caustic soda solution in the customary viscose-making process. Once such crumbs have been heat-ripened to the desired degree by the heat-

ripening treatment of the process hereof, they may be dissolved in relatively cold or refrigerated caustic soda solution at a temperature sufficiently low to arrest the heat-ripening reaction quickly or practically instantaneously and to yield a xanthate or viscose solution of the desired stability or keeping quality. The amount of the cold or refrigerated caustic soda solution thus used for dissolving the heat-ripened xanthate crumbs and the causticity of such solution may be such as to yield a finished xanthate or viscose solution of the desired cellulose content and causticity, for instance, such as is desired for spinning into rayon filaments.

- 5 10 15 20 25 30 35 40 45 50
- While not limited thereto, the present invention will now be described in terms of particular examples of procedure designed to yield finished cellulose xanthate or viscose solutions of a composition and other characteristics ordinarily desired for spinning into rayon filaments. According to one procedure, which involves preparing from wood pulp of low solution viscosity a cellulose xanthate solution by a single mixing and reacting operation, as disclosed in Richter Patent No. 2,112,576, a cellulose xanthate or viscose solution was prepared at cellulose and caustic soda concentrations much higher than desired in the finished viscose solution. Specifically, the solution thus prepared had a cellulose content of 12% and a caustic soda content of 10.86%. Such comparatively concentrated viscose solution was promptly after preparation heated indirectly in a tank, which was jacketed by a heating medium, and stirred or mixed constantly as it was being heated. The rate of heating was such that the viscose solution gradually rose from room temperature (about 18° C.) to a temperature of 50° C. after the first 20 minutes and to a temperature of 53° C. after the second 20 minutes, which latter temperature was maintained for 4 minutes with continued stirring of the solution. The resulting heat-ripened and concentrated viscose solution was then diluted immediately with refrigerated water at a temperature of 1° C., which water was added in amount calculated to dilute the solution to the desired final composition, namely, a cellulose content of 7.4% and a caustic soda content of 6.7%. The dilution of the solution was effected with constant stirring of the refrigerated diluting water and cellulose xanthate solution; and it was noted that, when the diluted solution had acquired substantial uniformity throughout, its temperature had dropped to 4° C. The ripeness value of the diluted solution at 4° C., as determined by a stand-

ard so-called ammonium chloride test, was found to be 11.2. Upon permitting the solution to stand exposed overnight to an atmosphere of 10° to 15° C., it was found that the ripeness value of the solution as determined by the standard ammonium chloride test, was 10.8. In other words, the diluted viscose solution had been practically stabilized in its ripeness and could be kept for a substantial period of time, that is, for many hours, with practically no change in its degree of ripeness. The normal or satisfactory ripeness value of viscose solution for spinning into rayon filaments ranges from 9 to 11, such value being determined by the same standard ammonium chloride test, which is described on page 15 334 in the 1926 edition of "Die Kunstseide" by V. Hottenroth.

A heat-ripened viscose solution prepared and stabilized by the procedure just described is quite suitable for spinning into rayon filaments. Thus, 20 the solution resulting from such procedure is clear and its ripeness falls into the range usually considered satisfactory for rayon manufacture. Again, the composition of such solution comports with that considered satisfactory for usual rayon manufacture; and the ripeness-stability of such 25 solution is such as to enable its storage or keeping for such substantial periods of time as are customary in usual viscose-rayon manufacture. It is thus seen that the present invention makes possible an accelerated or heat-ripening of viscose and at the same time the attainment of a finished viscose solution as satisfactory in practically every respect for viscose-rayon manufacture as the ripened viscose syrup heretofore prepared by prolonged ripening of a freshly prepared viscose solution at the final or adjusted cellulose and caustic soda concentrations.

Another example of procedure performed accordant with the present invention involved the 40 heat-ripening of cellulose xanthate crumbs prepared as ordinarily by xanthating soda-cellulose crumbs with carbon bisulphide in the usual xanthating drum. It might be mentioned, however, that the soda-cellulose crumbs thus xanthated were produced from a hardwood sulphite pulp rather than a spruce sulphite pulp. The xanthated crumbs, which were of characteristic orange color, were tumbled in a closed container submerged in a liquid heating medium maintained at a temperature of 50° C. As the tumbling of the solid xanthate crumbs continued, 45 their temperature, which was initially 27° C., gradually rose in 10 minutes to 37° C., in 20 minutes to 42° C., in 35 minutes to 48° C., and in 50 minutes to 50° C. The container was then opened and its content of heat-ripened xanthate crumbs discharged into a caustic soda solution of 4.89% caustic soda content and refrigerated to -2° C., which solution was used in amount calculated to yield a finished xanthate or viscose solution of 7.4% cellulose content and 6.7% caustic soda content. The mixing of the crumbs and the solution was effected in a high-speed mixing vessel, which quickly yielded a mixture at a temperature of 2° C. The crumbs went into solution gradually and about 90 minutes of continuous mixing were consumed before a clear solution, that is, one practically devoid of visible undissolved residue, was realized. The resulting 70 solution, which at 2° C. was found to have an ammonium chloride ripeness value of 10.9, was mixed for another 30 minutes and then permitted to stand overnight while exposed to a surrounding atmosphere at 10 to 15° C. An

ammonium chloride ripeness test made on the solution after overnight standing showed a value of 10.8, which value means that the solution had the desired ripeness-stability or keeping quality over a substantial period of time. The resulting viscose solution was thus of a ripeness and of a composition normal for spinning into rayon filaments. In saying that its ripeness or maturity was normal, it is meant that its ripeness value, as determined by the standard ammonium chloride test, fell within a range of 9 to 11; and in saying that its composition was normal, it is meant that its cellulose content fell within a range of about 6 to 8% and that its caustic soda content was approximately equal to, or in the neighborhood of, its cellulose content.

The practice of the present invention lends itself to various changes or modifications, including the incorporation into the cellulose xanthate or viscose solution of substances that increase the rate of the heat-ripening reaction and/or of substances that decrease the rate of the heat-ripening reaction. Thus, we have found that the addition of glycerine to a viscose solution accelerates its ripening even in the absence of heating and that the addition to a viscose solution of a very small amount of glycerine before it undergoes the heat-ripening and dilution treatments hereof permits a given degree of ripeness 30 to be attained in a distinctly shorter period of time than otherwise possible. On the other hand, we have found that neutral sodium sulphite decreases the rate of the ripening reaction and that the addition to a viscose solution of a very small amount of sodium sulphite prior to the heat-ripening and dilution treatments hereof may be desirable in order to decelerate the heat-ripening reaction to some extent. Again, sodium sulphite may to advantage be added to the refrigerated diluting water or caustic soda solution used to arrest the ripening reaction in the heat-ripened xanthate crumbs; or a very small amount of sodium sulphite may be added in crystalline or 35 concentrated solution form to the heat-ripened viscose solution before its dilution with the refrigerated water. In all such cases, the sodium sulphite serves to supplement the action of the cold aqueous medium in arresting quickly the ripening reaction in the viscose or cellulose xanthate solution and in enabling the realization of a finished viscose or cellulose xanthate solution of the desired ripeness-stability. In some instances, the glycerine may be added to the initial viscose 40 solution in order to increase the rate of the heat-ripening reaction thereupon, whereupon, when the heat-ripening reaction in the solution is to be arrested, sodium sulphite may be used, as hereinbefore described, in addition to the refrigerated aqueous medium to arrest the ripening reaction quickly at the desired stage of ripeness. Assuming that a finished viscose solution of 7.4% cellulose content and 6.7% caustic soda content is to be prepared, as hereinbefore described, one 45 may, if desired, use, say, about 1% of glycerine in the heat-ripening treatment and use in addition to the refrigerated aqueous medium, say, about 0.2% to 0.5% of sodium sulphite for the purpose of arresting the heat-ripening reaction in the xanthate solution and thus stabilizing the ripeness of the solution, the percentages of the glycerine and sodium sulphite being based on the finished viscose solution.

In speaking in the foregoing specification and 50 in the appended claims about heating cellulose

xanthate of a cellulose content greater than that of the finished solution desired or to be produced by the process hereof, we mean that the cellulose xanthate is heated either in the form of a solution more concentrated in cellulose than the finished solution or in the form of cellulose xanthate crumbs. When the cellulose xanthate is heat-ripened in the form of a viscose solution comparatively concentrated in cellulose, its causticity may be and preferably is such as to furnish all the caustic soda necessary for the finished solution; or some caustic soda may be supplied along with the refrigerated diluting water when the heat-ripened viscose solution is stabilized in its ripeness and brought to the desired final composition. On the other hand, when the cellulose xanthate is heat-ripened in the form of crumbs, practically all of the caustic soda necessary for dissolving the crumbs and furnishing a finished viscose solution of the desired composition may be supplied along with the refrigerated water used to arrest the heat-ripening reaction in the crumbs. In any event, the aqueous medium used to arrest quickly any further substantial ripening reaction in the xanthate, whether in the form of a heat-ripened viscose solution or of crumbs, is admixed with the xanthate in the presence of sufficient caustic soda or equivalent alkali to permit the desired substantially complete dissolution of the xanthate and to yield a finished xanthate solution of the desired composition and ripeness-stability.

Irrespective of whether comparatively concentrated viscose solutions or cellulose xanthate crumbs are subjected to the heat-ripening treatment thereof, it is usually desirable for such purposes as manufacturing rayon filaments and films that the finished solution to be spun into rayon filaments or cast into films be of a cellulose content of about 6 to 8%, that is, that the ripened solution be of a cellulose content of about 6 to 8% after it has been diluted with refrigerated aqueous medium and cooled thereby to a temperature, say, downwards of about 15° C., at which substantial ripeness-stability of solution prevails over a substantial period of time, namely, a period of greater than, say, about 12 hours. So, too, the causticity of the finished viscose solution should be such as to promote or maintain substantially complete solution of the cellulose xanthate. A caustic soda content or causticity in the finished viscose solution approximately equal to, or in the neighborhood of, that of the cellulose content of the solution makes possible the realization of the last-named desideratum. It is, however, to be understood that the process hereof, although advantageously applicable to the preparation of finished viscose solutions designed especially for such purposes as manufacturing rayon filaments and films, may be extended to the preparation of finished viscose or cellulose xanthate solutions of a cellulose content above or below the range of about 6% to 8% and of a causticity or caustic soda content preferably approximating the cellulose content and in any event sufficient to promote or maintain substantially complete solution of the cellulose xanthate.

We claim:

1. A process of producing a solution of heat-

- ripened cellulose xanthate having a desired degree of ripeness, which comprises heating to much higher than room temperature and in admixture with glycerine a cellulose xanthate of a cellulose content greater than that of said solution to be produced, said glycerine amounting to about 1%, based on said solution, continuing such heating until said xanthate has acquired substantially the degree of ripeness desired, and mixing with 5 said heated xanthate and refrigerated aqueous medium in amount sufficient to dilute the cellulose content of said xanthate to that of the solution to be produced and about 0.2% to 0.5% sodium sulphite, based on said solution, said aqueous medium being sufficiently refrigerated to arrest quickly further substantial ripening reaction in said xanthate and to cool the mixture to a temperature at which said xanthate has substantial ripeness-stability over a substantial 10 period of time and said aqueous medium being mixed with said xanthate in the presence of sufficient alkali to promote substantially complete dissolution of said xanthate in said aqueous medium.
2. A process of producing a heat-ripened viscose solution having a desired degree of ripeness, which comprises heating to much higher than room temperature a viscose solution containing glycerine and having a cellulose content greater than that of said solution to be produced, said glycerine amounting to about 1%, based on said solution, continuing such heating until said solution has acquired substantially the degree of ripeness desired, and mixing with said heated 15 solution refrigerated water in amount sufficient to dilute the cellulose content of said solution to that of the solution to be produced, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
3. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 20 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
4. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 25 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
5. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 30 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
6. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 35 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
7. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 40 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
8. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 45 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
9. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 50 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
10. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 55 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
11. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 60 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.
12. A process of producing a heat-ripened viscose solution having a desired degree of ripeness, which comprises heating to much higher than room temperature a viscose solution of a cellulose content greater than that of the solution to be produced, continuing such heating until said solution has acquired substantially the degree of ripeness desired, and mixing with said heated 65 solution refrigerated aqueous medium in amount sufficient to dilute the cellulose content of said solution to that of the solution to be produced and about 0.2% to 0.5% sodium sulphite, based on said solution, said water being sufficiently refrigerated to arrest quickly further substantial ripening reaction in said solution and to cool said solution to a temperature at which it has substantial ripeness-stability over a substantial period of time and said water being mixed with said viscose solution in the presence of sufficient alkali to maintain the viscose substantially completely dissolved.

GEORGE A. RICHTER.  
HAROLD P. VANNAH.